

# United States Patent [19]

Szieleit

[11] 3,816,313

[45] June 11, 1974

[54] **LUBRICANT PROVIDING IMPROVED FATIGUE LIFE**

[75] Inventor: **Hans J. Szieleit, Sarnia, Ontario, Canada**

[73] Assignee: **Esso Research and Engineering Company, Linden, N.J.**

[22] Filed: **Nov. 17, 1972**

[21] Appl. No.: **307,492**

[52] U.S. Cl. .... **252/49.6, 260/448.8 R**

[51] Int. Cl. .... **C10m 1/50**

[58] Field of Search..... **252/49.6; 260/448.8 R**

## [56] References Cited

### UNITED STATES PATENTS

2,780,636 2/1957 Wright et al. .... **252/49.6 X**

|           |        |                      |            |
|-----------|--------|----------------------|------------|
| 2,897,222 | 7/1959 | Bailey .....         | 252/49.6 X |
| 2,947,772 | 8/1960 | Eynon et al. ....    | 252/49.6 X |
| 2,995,591 | 8/1961 | Kovacich et al. .... | 252/49.6 X |
| 3,098,825 | 7/1963 | Shiffter .....       | 252/49.6 X |

Primary Examiner—W. Cannon

Assistant Examiner—W. Cannon

[57]

## ABSTRACT

The fatigue life of a lubricant composition, particularly one designed for the lubrication of bearings having rolling elements, is markedly improved by incorporating therein a condensation polymer of an alkyl trialkoxy silane or of an alkoxyalkyl trialkoxy silane.

**9 Claims, No Drawings**

# LUBRICANT PROVIDING IMPROVED FATIGUE LIFE

## BACKGROUND OF THE INVENTION

There has been a need for a lubricant that will prolong the life of bearings by reducing the tendency of metal bearing components to fail as a result of fatigue caused by repeated stress. This is particularly a problem in rolling contact bearings. See for example "Some Effects of Additives on Rolling Contact Fatigue" by Fred G. Rounds, ASLE Transactions, Volume 10, pages 243-255 (1967).

## REFERENCES TO THE PRIOR ART

It is known to use alkoxy silanes as hydraulic fluids and lubricants. See for example U.S. Pat. Nos. 2,947,772, 2,985,678 and 2,995,590. The use of homopolymers of vinyl alkoxy silanes, polymerized through the vinyl groups, as foam suppressors in concentrations of from 2 to 50 parts per million in hydrocarbon oils is taught in U.S. Pat. No. 2,862,885. No prior art is known on the use of condensation polymers of alkoxy silanes as additives capable of increasing the fatigue life of a lubricant composition.

## DESCRIPTION OF THE INVENTION

In accordance with the present invention it has been found that exceptional antifatigue qualities are imparted to a hydrocarbon lubricant by incorporating therein from about 0.01 to about 5 weight percent of the condensation polymer of an alkyl trialkoxy silane or of an alkoxyalkyl trialkoxy silane. The monomer from which the condensation polymer is derived can be represented by the formula:



wherein R is C<sub>1</sub> to C<sub>24</sub> alkyl or C<sub>2</sub> to C<sub>24</sub> alkoxyalkyl, preferably C<sub>3</sub> to C<sub>18</sub> alkyl or alkoxyalkyl, and R' is C<sub>1</sub> to C<sub>12</sub> alkyl or C<sub>2</sub> to C<sub>12</sub> alkoxyalkyl, preferably C<sub>4</sub> to C<sub>8</sub> alkyl or alkoxyalkyl. By alkoxyalkyl is meant an ether group that can be represented by C<sub>n</sub>-O-C<sub>m</sub>- where the sum of n plus m is 2 to 24 in the case of R and 2 to 12 in the case of R'. Representative monomers include dodecyl tributoxy silane, decyl tripropoxy silane, ethoxy propyl triheptoxy silane, octadecyl tripenoxy silane, methoxyamyl trihexoxy silane, hexyl tridecoxyl silane, and octyl tri(methoxypropyl oxy) silane. One method for preparing alkyl trialkoxy silanes is to react one mole of a commercially available alkyl trichloro silane with 3 moles of an aliphatic alcohol. See for example U.S. Pat. Nos. 2,947,772 and 2,995,590.

The additives of the present invention are condensation polymers of the above-noted alkoxy silanes and can be represented by the formula:



wherein x is from about 1 to about 60, or more usually from about 1 to about 40. Usually the additive will comprise a mixture of condensation polymers so that x will represent an average which will usually not be a whole number. The average molecular weights of these additives will be within the range of about 300 to about 30,000. More generally additives with average molecular weight ranging from about 500 to 10,000 will be used.

A condensation polymer can be obtained by refluxing an alkyl trialkoxy silane with water in the presence of a strong acid catalyst which is preferably HCl because of its ease of removal from the reaction mixture. The extent of condensation will depend somewhat on the proportion of water to alkoxy silane; thus in theory one mole of water and two moles of alkoxy silane should give principally the dimer in accordance with the equation:



Higher polymers would require slightly greater proportions of water.

The condensation polymers can also be formed directly by reaction of an appropriate sodium alcoholate with an appropriate halogenated silane. Thus one mole of octadecyl trichlorosilane will react with 3 moles of sodium pentoxyde at ambient temperature to give a condensation polymer of octadecyl tripentoxyl silane with sodium chloride as a by-product. Similarly one mole of 3-chloropropyl trichlorosilane will react with 4 moles of sodium pentoxyde to give a condensation polymer of pentoxypropyl tripenoxy silane.

The alkoxy silane condensation polymers employed in the present invention will be used in lubricant compositions in amounts ranging from about 0.01 to about 5 percent by weight based on the total composition. Preferably they will be used within the range of from about 0.1 to about 2 percent by weight. The lubricating oils to which the additives can be added include not only mineral lubricating oils but synthetic oils also. The mineral lubricating oils can be of any preferred type, including those derived from the ordinary paraffinic, naphthenic, asphaltic, or mixed base mineral crude oils by suitable refining methods. The synthetic lubricating oils include not only hydrocarbon oils but also ester oils such as di-2-ethylhexyl sebacate, polyglycols, polycarbonates, glycol esters such as C<sub>13</sub> oxo acid diesters of tetraethylene glycol, and complex esters such as the complex ester formed by reacting one mole of sebacic acid with 2 moles of tetraethylene glycol and 2 moles of 2-ethylhexanoic acid.

In the lubricant compositions, other conventional additives may also be present, including dyes, pour point depressants, antiwear agents, e.g., tricresyl phosphate, zinc dialkyl dithiophosphates of 3 to 8 carbon atoms, antioxidants such as phenyl-alpha-naphthylamine, tert. octylphenol sulfide, bisphenols such as 4,4'-methylene bis(2,6-di tert. butylphenol), viscosity index improvers

such as polymethacrylates, polyisobutylene, alkyl fumarate-vinyl acetate copolymers, ashless dispersants or detergents, e.g., the reaction product of tetra-ethylene pentamine and polyisobutyl succinic anhydride. Antioxidants, rust inhibitors and antiwear additives are particularly useful. The lubricant compositions include not only liquid compositions but lubricating greases as well. Thus the compositions can contain grease thickeners including metal soaps, metal salts, talc, carbon black, etc.

The nature of this invention and the advantages arising from its use will be more fully understood when reference is made to the ensuing examples which include preferred embodiments.

15

#### EXAMPLE 1

##### Preparation A — Polymer of Octadecyl Tri-n-Amoxy Silane

To a mixture of 1/10 mol sodium n-amoxide in 2/10 mol of amyl alcohol and approximately 10 ml of petroleum ether, 1/30 mol of octadecyl trichloro silane was added dropwise under stirring at room temperature over a period of about 20 minutes. The product, octadecyl tri-n-amoxy silane, was separated from the by-product, sodium chloride, by three successive extractions with 10 ml each of petroleum ether. The petroleum ether solvent was then distilled off. The mixture of sodium n-amoxide in amyl alcohol used in this preparation was prepared by adding 1/10 mol of sodium methoxide as a 10/1 solution in methanol to 3/10 mol of amyl alcohol.

In separate preparations of the condensation polymer following the above procedure the average molecular weights varied from about 1,000 to about 3,100.

##### Preparation B — Condensation Polymer of iso-Amoxy Propyl Tri iso-Amoxy Silane

To a mixture of 0.56 mol of sodium iso-amoxide, 0.5 mol isoamylalcohol and 300 ml petroleum ether, 0.175 mol of 3-chloropropyl trichlorosilane was added dropwise under stirring at room temperature, over a period of about 20-25 minutes. The resulting product was extracted with petroleum ether as in Preparation A, and the petroleum ether solvent was then distilled off.

The average molecular weights of condensation polymers prepared by the above procedure ranged from about 560 to about 1,440 if care was taken to dry the reactants. Without such care the molecular weight was found to be considerably higher.

##### Preparation C — Condensation Polymer of Ethoxypropyl Tri-iso-Amoxy Silane

A 1/10 mol quantity (19.9 g) of 3-chloropropyl trimethoxy silane was added dropwise with stirring at room temperature to 1/10 mol of sodium ethoxide as a 10/1 solution in ethanol. To complete the reaction, the mixture was refluxed for 2 hours and the sediment (NaCl) removed by filtration. The excess ethanol was distilled off under vacuum. 40 g (0.45 mol) of iso-amyl alcohol and two drops of a compound which released hydrogen chloride (chloro methyl trimethyl silane) were added and the mixture refluxed for 2 hours. The liberated methanol and the excess iso-amyl alcohol were distilled off. The molecular weight of the resulting product was  $828 \pm 10$  percent, indicating the probable formation of the trimer.

##### Preparation D — Condensation Polymerization of Ethoxypropyl Tri iso-Amoxy Silane (ETAS)

A mixture of 1.5 ml of 10 percent aqueous HCl and 20 g ETAS (MW:828) was refluxed for 2 hours. The liberated iso-amyl alcohol was distilled off under vacuum (ca 1 to 2 mm Hg). The yield was 11.4 g of the condensed version of ETAS having an average molecular weight of  $3,510 \pm 10$  percent. This would correspond to approximately 15.5 units of



15

per molecule.

##### Preparation E — Condensation Polymer of Methoxypropyl Tri-iso-Octoxy Silane

The procedure of Preparation C was followed, but employing sodium methoxide in place of sodium ethoxide and iso-octyl alcohol in place of iso-amyl alcohol. No determination of the molecular weight of the condensation polymer was made.

#### EXAMPLE 2

Lubricating oil blends were prepared using either a base oil X, which was an SAE 10 grade, phenol extracted, dewaxed and hydrofinned lube distillate from a Western Canadian crude oil, or a base oil Y, which was a refined SAE 10 grade multipurpose hydraulic oil containing a pour point depressant (0.7 vol. percent of a mixture of wax-alkylated naphthalene and methacrylate ester concentrate) an oxidation inhibitor (0.3 wt. percent 2,6-di-tert. butyl p-cresol) an antiwear agent (0.5 vol. percent of dihydrocarbyl dithio-phosphate) and a rust inhibitor (0.05 vol. percent of a 50 percent oil concentrate of neutral barium dinonyl naphthalene sulfonate plus 0.04 vol. percent of ethylene oxide treated tetrapropenyl succinic acid). The blends were prepared by adding, by simple mixing, various concentrations of condensation polymers of alkoxy silanes prepared by the procedures described above. Various concentrations and molecular weights were used in the different blends. Each of the blends as well as each of the base oils was subjected to a test designed to determine the effect of the oils on the fatigue life of bearings. This test is known to correlate with actual field results. The test machine used was a rolling four-ball machine in which three steel balls are allowed to roll freely in a conforming race, while a fourth steel ball which is held firmly in a chuck is pressed on the top of the other three balls and rotated under load. The speed of rotation was 1,600 rpm and the applied load was 887 pounds, which corresponds to an initial maximum contact stress of  $1.07 \times 10^6$  psi. To run the test the required amount of test oil was poured into the reservoir and the equipment was brought up to the test temperature of 150° F. Each test was run until one of the balls developed a fatigue spall. The excessive vibrations that resulted from the failure of one of the balls actuated a vibration switch which automatically turned off the machine. The longer the time period to failure the greater are the antifatigue properties of the oil being tested. The results obtained, in terms of millions of revolutions until failure, are shown in Table I which follows:

TABLE I

| Oil Tested | Weight % Additive | Average Mol. Wt. of Additive | Mean Fatigue Life $\times 10^6$ Rev. |
|------------|-------------------|------------------------------|--------------------------------------|
| Base Oil X | —                 | —                            | 0.44                                 |
| Oil X + B  | 0.15              | 8000                         | 1.58                                 |
| Base Oil Y | —                 | —                            | 1.1                                  |
| Oil Y + A  | 0.5               | 1010                         | 2.2                                  |
|            | 0.5               | 3100                         | 2.7                                  |
| Oil Y + B  | 0.05              | 8000                         | 1.3                                  |
|            | 0.10              | 8000                         | 2.0                                  |
|            | 0.15              | 8000                         | 3.3                                  |
|            | 0.20              | 8000                         | 3.8                                  |
| Oil Y + C  | 0.5               | 828                          | 2.4                                  |
| Oil Y + D  | 0.1               | 3510                         | 2.7                                  |
| Oil Y + E  | 0.3               | —                            | 2.2                                  |

It will be noted that in each instance the mean fatigue life of the lubricating oil was increased by the addition of an alkoxy silane condensation polymer. The data show that at a given concentration of additive an increase in molecular weight effects an improvement in anti-fatigue properties and that with an additive of a given molecular weight, fatigue life increases with increased concentration of the additive in the composition.

### EXAMPLE 3

Using a conventional procedure, a lubricating grease is prepared from 76 parts of weight of 12-hydroxystearic acid, 11.5 parts of lithium hydroxide monohydrate, and 908 parts of a solvent-refined mineral lubricating oil of about 460 SUS viscosity measured at 100° F. To prepare the grease, the 12-hydroxystearic acid is added to about half of the total oil used in the complete grease, the mixture is heated to about 190°-200° F., the lithium hydroxide is added in the form of an aqueous solution, and the resulting mixture is then heated with stirring to a final temperature of about 380°-390° F. Then the remaining portion of the base oil is stirred in and the mixture is cooled to ambient temperature. When cooling has reached about 100° F. during cooling, 5 parts of 1,010 molecular weight condensation polymer of octadecyl tri-n-amoxy silane (Preparation A of Example 1) is added and the grease is milled in a conventional grease mill.

It will be understood that there is no intention that

the scope of this invention be limited to the foregoing specific examples which have been presented merely as illustrative of the invention.

What is claimed is:

- 5 1. A lubricating oil composition comprising a major proportion of a hydrocarbon lubricating oil to which has been added from about 0.01 to about 5 percent by weight of the condensation polymer of an alkyl or alkoxyl alkyl trialkoxy silane, said condensation polymer being represented by the formula:



wherein X is from about 1 to about 60, R is C<sub>1</sub> to C<sub>24</sub> alkyl, or alkoxy alkyl totaling 2 to 24 carbon atoms, and R' is C<sub>1</sub> to C<sub>12</sub> alkyl, or alkoxy alkyl totaling 2 to 12 carbon atoms.

20 2. Composition as defined by claim 1 wherein X is from about 1 to about 40.

3. Composition as defined by claim 1 wherein said condensation polymer has an average molecular weight of from about 300 to about 30,000.

25 4. Composition as defined by claim 1 wherein said condensation polymer is that of octadecyl tri-n-amoxy silane.

5. Composition as defined by claim 1 wherein said condensation polymer is that of isoamoxypropyl tri-isoamoxypropyl silane.

30 6. Composition as defined by claim 1 wherein said condensation polymer is that of methoxypropyl tri-octoxy silane.

7. Composition as defined by claim 1 wherein said condensation polymer is that of ethoxypropyl tri-isoamoxypropyl silane.

35 8. Composition as defined by claim 1 which additionally contains a grease thickener.

9. Composition as defined by claim 1 which additionally contains at least one additive selected from the group consisting of an antioxidant, a rust inhibitor and an antiwear additive.

45 \* \* \* \* \*